

## UNITED STATES PATENT OFFICE

2,069,805

CELLULOSIC STRUCTURES AND METHODS  
FOR PRODUCING SAMEWinfield Walter Heckert, Ardentown, Del., as-  
signor, by mesne assignments, to E. I. du Pont  
de Nemours & Company, Wilmington, Del., a  
corporation of DelawareNo Drawing. Application September 15, 1934,  
Serial No. 744,258

8 Claims. (Cl. 106—40)

This invention relates to cellulosic structures such as filaments, threads, fabrics, sheets, films, caps, tubing, or the like. More particularly, this invention relates to cellulosic structures of 5 the type just mentioned having a subdued or low luster or that are more or less opaque.

In the ordinary methods of preparing cellulosic structures, such as filaments, threads, films, caps, tubing, etc., from viscose, cupram- 10 monium, nitrocellulose, cellulose acetate and other cellulosic solutions (without the addition of opaques or low luster-inducing agents to the solutions), the products are transparent or translucent or very highly lustrous. For many pur- 15 poses, transparency, brilliant sheen and luster are not desirable and thus restrict the uses of the materials. Recently, various methods have been proposed for producing cellulosic structures having a low or subdued luster or opacity.

20 I have found that I can produce cellulosic structures characterized by a low luster or opacity by incorporating therein a tertiary amine of the character described in detail hereinafter which imparts opacity or low luster by remain- 25 ing in the cellulosic structure.

An object of the invention comprises the production of new opacified or low luster cellulosic structures. A further object of the invention relates to the production of novel cellulosic 30 structures containing organic compounds which remain in the finished article and which impart opacity or low luster. Other objects of the invention will appear hereinafter.

The objects of the invention are accomplished 35 in general by incorporating in the cellulosic solution from which the structure is to be produced an opaques or a low luster-inducing agent of the type hereinafter more fully explained.

The low luster-inducing agent contemplated 40 by this invention is an organic compound of high molecular weight having a tertiary amine grouping and comprising two or more carbocyclic or heterocyclic nuclei highly deficient in hydrogen.

So far as the instant invention is concerned, 45 each closed chain of carbon or hetero- atoms or combination of carbon and hetero- atoms will be considered a nucleus. Thus, benzene, naphthalene and carbazole have one, two, and three nuclei respectively.

These opaques or low luster-inducing agents, 50 which are preferably white in color, possess a sufficiently low vapor pressure and are sufficiently inert to resist the change or removal from the 55 cellulosic structure in the ordinary process of

making and finishing the same during the manufacture thereof. They also effectively resist removal or change during any of the usual processes to which the finished cellulosic structure may be subjected, such as boiling-off, dyeing, 5 bleaching, washing, ironing, etc. These substances are incompatible with the mass of the substance constituting the final product. They may be soluble but, in the preferred embodiment of this invention, they are insoluble in 10 the solution from which the structure is prepared.

Highly effective delusterants function in particular by reason of their opacifying power which is a function of the difference in refractive index between the delusterant particle and the 15 surrounding medium. Those in my preferred range differ from the index of the medium by at least 0.10 and the greater this difference, the more effective the compound as an opacifier or delusterant. Most organic compounds have several indexes and the statement just made refers to the highest index of the compound or to any 20 one of the several indexes.

As illustrative examples of tertiary amines coming within the scope of this invention are the 25 following:

|                                     |    |
|-------------------------------------|----|
| Dibenzyl aniline                    |    |
| Ethyl benzyl aniline                |    |
| Triphenyl amine                     |    |
| Ethyl diphenylamine                 | 30 |
| Methyl diphenylamine                |    |
| Dimethyl anthranylamine             |    |
| Phenyl-di- $\beta$ -naphthyl amine  |    |
| Dimethyl- $\alpha$ -naphthylamine   |    |
| Dimethyl- $\beta$ -naphthylamine    |    |
| Di-ethyl- $\alpha$ -naphthylamine   |    |
| Di-ethyl- $\beta$ -naphthylamine    |    |
| Ethyl-di- $\beta$ -naphthyl amine   |    |
| Benzyl-di- $\alpha$ -naphthyl amine |    |
| Diphenyl- $\alpha$ -naphthyl amine  | 35 |
| Phenyl-di-biphenyl amine            |    |
| Tetra-phenyl-ethylene diamine       |    |
| Tetra-phenyl-phenylene diamine      |    |
| Diphenyl benzthiazyl amine          |    |
| Phenyl difurfuryl amine             | 40 |
| Di-ethyl- $\alpha$ -naphthyl amine  |    |
| Methenyl diphenyl amine             |    |

The scope of this invention is not intended to include compounds the only tertiary nitrogen of 50 which is an amido nitrogen. In other words, the invention contemplates only true amines and not amides.

The organic compounds contemplated as de- 55 lusterants in accordance with the principles of

this invention are embraced in the following formula:



5 in which at least two carbocyclic or heterocyclic nuclei highly deficient in hydrogen are included, and in which  $R_1$ ,  $R_2$  and  $R_3$  are radicals other than hydrogen. One of the radicals may be 10 naphthyl, for example, in which event the other radicals need not contain a cyclic nucleus, or, alternatively, two or more of the radicals may contain a phenyl group or a substituted phenyl group. The cyclic nuclei may be attached directly 15 to the nitrogen atom, for example, as in triphenylamine, or some of them may be indirectly attached through the linkage of an alkyl group as in the case of benzyl-di-naphthyl amine. Where the other conditions are fulfilled, the invention 20 contemplates an N- attached radical which may be aliphatic (either saturated or unsaturated, e. g. alkyl or alkylene), an aromatic, aralkyl or alkaryl, alicyclic or heterocyclic. By way of illustrating specifically those radicals 25 which may be attached to the N atom of the tertiary amine, the following groups may be mentioned: e. g. methyl, phenyl, benzyl, or a heterocyclic group linked thru carbon or their colorless substitution products, such as their  $-R$ ,  $-O-R$ ,  $-S-R$ ,  $-Se-R$ ,  $-Te-R$ ,  $-NH-R$ ,  $-CO-R$ ,  $-SO_2-R$ ,  $-SO-R$ , hydroxy alkyl and halogen derivatives where "R" may be an alkyl, aryl, aralkyl, alkaryl, or a heterocyclic group.

Organic compounds of the character described 35 which have relatively high refractive indexes and which are preferred on the basis of cost, color stability, acid insolubility and effectiveness are the following:

40 Triphenyl amine  
Methenyl-diphenyl-diamine  
Phenyl-di-beta-naphthylamine  
Ethyl-di-alpha-naphthyl amine  
Benzyl-di-alpha-naphthyl amine  
Tetra-phenyl-phenylene diamine  
45 Tetra-phenyl-ethylene diamine  
Diphenyl- $\alpha$ -naphthyl amine

The quantity of the low luster-inducing or 50 opaques agent which may be used may vary within wide limits, depending principally upon the opaques and luster desired in the final product. Cellulosic structures containing these low luster-inducing or opaques agents in amounts ranging from 0.10-20.0% by weight have given 55 satisfactory results, but, of course, it is obvious that smaller or larger quantities may be employed as desired. When a viscose solution is employed, satisfactory results may be secured if it contains 7% cellulose and from 0.01-1.5% more or less of the low luster-inducing or opaques agent.

60 If desired, the low luster-inducing agents contemplated by the instant invention may be used in combination with each other or with other low luster-inducing agents, such as mineral oil, petroleum jelly, waxes, paraffin, benzene, toluene, pine oil or inorganic pigments, such as titanium oxide, lithopone, zinc sulfide, etc.

The low luster-inducing agent may be added 70 to the solution at any stage in the course of the manufacture thereof, or after the preparation of the solution and prior to the spinning, extrusion or casting operation. It may be added directly, if the particle size is satisfactory, or after suitable adjustment of the particle size by 75 any of the well known methods, such as emul-

sification, grinding in a colloid mill or pebble mill, or in the form of a suspension or emulsion prepared with or without the assistance of suitable dispersing agents or protective colloids, such as soaps, sulfonated oils, alkyl naphthalene sulfonates, sodium caseinate, etc. or combinations thereof.

In order to more fully explain the principles of this invention, the following illustrative examples are given:

10 *Example I.*—One hundred parts of molten di-benzyl aniline are emulsified with 400 parts of water containing 8 parts casein, 2.4 parts of hydrated sodium phosphate and 2 parts of Monopole oil by passing the mixture through a colloid 15 mill such as a Disper-mill at a temperature of 90° C. The resulting emulsion, consisting of droplets 1-4 microns in diameter, is cooled and incorporated in viscose containing 7% cellulose and 6% caustic soda in the proportion of 1 to 20. 20 This dispersion is ripened to the desired index and spun into rayon or cast into sheets. The resulting product has a desirable low luster.

25 *Example II.*—Four hundred parts of ethyl di-beta-naphthylamine (Berichte 20, 2619) are 25 ground with 8 parts of sodium caseinate and 592 parts of water in a ball mill until practically all the particles lie below 4 microns in diameter.

One per cent of this dispersion is incorporated 30 in viscose and, after ripening, the latter is spun into rayon. The product has a beautiful low luster similar to that obtained with inorganic pigments.

35 It is to be understood that these examples do not in any way restrict the invention thereto but merely illustrate several specific and preferred embodiments which have given satisfactory results.

Though the preferred embodiments of this invention contemplate the incorporation of the low 40 luster-inducing agent in the solution at some time prior to the extrusion or casting thereof, satisfactory results may be secured also by applying the low luster-inducing agent to a previously 45 formed cellulosic structure. In other words, the low luster-inducing agent may be incorporated in the final cellulosic structure by an after-treatment.

Though the invention has been specifically described in connection with the viscose process, it 50 is obvious that the principles thereof are equally applicable to the cuprammonium cellulose, cellulose nitrate, and cellulose acetate processes.

55 In the case of cellulosic solutions of wholly organic solvents, it is only necessary that a suitable choice of amine be made so that the solubility characteristics do not interfere. It has already been pointed out that the low luster-inducing substance must be incompatible with the mass of substance constituting the final product. In addition, in the case of cellulose acetate or nitrate spinning solutions, it is preferable that the low luster-inducing substances be insoluble in the solvent employed. However, resinous materials and certain crystallized substances soluble in the solvent, precipitate, on the evaporation of the solvent, in the cellulose acetate in the form of fine amorphous or crystalline particles sufficiently small and well distributed to avoid harmful effect on the physical properties of the resulting structure. The advantage in such cases lies in avoiding the necessity for emulsifying or grinding the compounds to obtain suitable subdivision. Suitable compounds may be readily 60 65 70 75 80 85 90 95

selected from any specific system by one skilled in the art.

While the invention has been described generally with respect to the use of the various compounds mentioned herein in opaquing cellulosic structures prepared by casting or spinning methods, it is desired to emphasize the fact that these compounds are of special benefit in the spinning of artificial silk. Thus, undelustered artificial silk has a shade and luster which is undesired for a great many purposes. In accordance with the present invention, it is possible to produce artificial silk, particularly of the regenerated cellulose type prepared from viscose or cuprammonium cellulose, having a pleasing dull appearance, the dullness being of any degree desired, in which the opaquing or delustering agent is uniformly distributed and which does not interfere with the tenacity of the yarn to any large extent.

Since it is obvious that various changes and modifications may be made in the above description without departing from the nature or spirit thereof, this invention is not restricted thereto except as set forth in the claims.

I claim:

1. Delustered cellulosic articles prepared from cellulosic solutions containing, in a phase distinct from that of the cellulosic material therein a finely divided, white delustering agent comprising a polycyclic tertiary amine, said amine having a refractive index which differs from the refractive index of the surrounding medium by at least 0.1.
2. Delustered cellulosic articles prepared from cellulosic solutions containing, in a phase distinct from that of the cellulosic material therein, a finely divided, white delustering agent comprising a tertiary amine having at least two cyclic nuclei, at least one of said nuclei being directly attached to the nitrogen atom of the amine, said amine having a refractive index which differs from the refractive index of the surrounding medium by at least 0.1.
3. Delustered cellulosic articles prepared from cellulosic solutions containing, in a phase distinct from that of the cellulosic material therein, a finely divided, white delustering agent comprising a tertiary amine having at least two cyclic nuclei directly attached to the nitrogen atom of the amine, said amine having a refractive index which differs from the refractive index of the surrounding medium by at least 0.1.
4. Delustered cellulosic articles prepared from cellulosic solutions containing, in a phase distinct from that of the cellulosic material therein, a finely divided, white delustering agent comprising

a tertiary amine taken from the class consisting of dibenzyl aniline, ethyl benzyl aniline, triphenyl amine, ethyl diphenylamine, methyl diphenylamine, dimethyl anthranylamine, phenyl-di- $\beta$ -naphthyl amine, dimethyl- $\alpha$ -naphthylamine, dimethyl- $\beta$ -naphthylamine, di-ethyl- $\alpha$ -naphthylamine, di-ethyl- $\beta$ -naphthylamine, ethyl-di- $\beta$ -naphthyl amine, benzyl di- $\alpha$ -naphthyl amine, diphenyl- $\alpha$ -naphthyl amine, phenyl-di-bi-phenyl amine, tetra-phenyl-ethylene diamine, tetra-phenyl-phenylene diamine, diphenyl benzthiazyl amine, phenyl difurfuryl amine, di-ethyl- $\alpha$ -naphthyl amine, methenyl diphenyl diamine.

5. Delustered regenerated cellulose articles containing, in a phase distinct from that of the regenerated cellulose, a finely divided, white delustering agent comprising a polycyclic tertiary amine, said amine having a refractive index which differs from the refractive index of the surrounding medium by at least 0.1.

10. Delustered regenerated cellulose articles containing, in a phase distinct from that of the regenerated cellulose, a finely divided, white delustering agent comprising a tertiary amine having at least two cyclic nuclei, at least one of said nuclei being directly attached to the nitrogen atom of the amine, said amine having a refractive index which differs from the refractive index of the surrounding medium by at least 0.1.

15. Delustered regenerated cellulose articles containing, in a phase distinct from that of the regenerated cellulose, a finely divided, white delustering agent comprising a tertiary amine having at least two cyclic nuclei directly attached to the nitrogen atom of the amine, said amine having a refractive index which differs from the refractive index of the surrounding medium by at least 0.1.

20. Delustered regenerated cellulose articles containing, in a phase distinct from that of the regenerated cellulose, a finely divided, white delustering agent comprising a tertiary amine having at least two cyclic nuclei directly attached to the nitrogen atom of the amine, said amine having a refractive index which differs from the refractive index of the surrounding medium by at least 0.1.

25. Delustered regenerated cellulose articles containing, in a phase distinct from that of the regenerated cellulose, a finely divided, white delustering agent comprising a tertiary amine taken from the class consisting of dibenzyl aniline, ethyl benzyl aniline, triphenyl amine, ethyl diphenylamine, methyl diphenylamine, dimethyl anthranylamine, phenyl-di- $\beta$ -naphthyl amine, dimethyl- $\alpha$ -naphthylamine, dimethyl- $\beta$ -naphthylamine, di-ethyl- $\alpha$ -naphthylamine, di-ethyl- $\beta$ -naphthylamine, ethyl-di- $\beta$ -naphthyl amine, benzyl di- $\alpha$ -naphthyl amine, diphenyl- $\alpha$ -naphthyl amine, phenyl-di-bi-phenyl amine, tetra-phenyl-ethylene diamine, tetra-phenyl-phenylene diamine, diphenyl benzthiazyl amine, phenyl difurfuryl amine, di-ethyl- $\alpha$ -naphthyl amine, methenyl diphenyl diamine.

WINFIELD WALTER HECKERT.